

## UNITED STATES PATENT OFFICE.

ZAY JEFFRIES, OF CLEVELAND HEIGHTS, AND ROBERT S. ARCHER, OF EAST CLEVELAND, OHIO, ASSIGNORS TO ALUMINUM COMPANY OF AMERICA, OF PITTSBURGH, PENNSYLVANIA, A CORPORATION OF PENNSYLVANIA.

## MAKING CASTINGS OF ALUMINUM ALLOYS.

To Drawing.

Application filed January 4, 1921. Serial No. 435,024.

To all whom it may concern:

Be it known that we, ZAY JEFFRIES and ROBERT S. ARCHER, both citizens of the United States of America, residing at Cleveland Heights and East Cleveland, respectively, in the county of Cuyahoga and State of Ohio, have invented certain new and useful Improvements in Making Castings of Aluminum Alloys, of which the following is a full, clear, and exact description.

This invention relates to the production of aluminum alloy castings particularly castings made of alloys containing silicon or copper or both, with or without other metals, and its chief object is to provide a simple and effective method which will produce light-weight castings with a hitherto unobtainable combination of physical properties, especially as regards elastic limit, tensile strength and ductility. To this and other ends the invention consists in the novel method hereinafter described.

As will be seen from the subjoined description, the invention is based upon the combination of certain steps, some of them novel with us, and in part the invention resides in the discovery that certain alloys are especially susceptible to improvement by heat treatment after casting, and that certain methods of casting such alloys further and peculiarly adapt them to such treatment; and in the additional discovery of temperature and duration of heat treatment in combinations appropriate to the particular alloys and methods of casting involved. With the aid of these discoveries we have been able to produce castings having improved physical properties with respect to elastic limit, tensile strength and ductility to an extent hitherto unattainable, with the result that it is now possible to use aluminum alloy castings for purposes for which their use has previously been impracticable.

It has been found that the addition of a substantial amount of silicon to aluminum alloys very materially improves their casting qualities, thus rendering it possible to successfully and easily make castings which would otherwise be very difficult to produce.

In particular, the presence of a substantial amount of silicon enables us to produce alloys having excellent casting qualities, even better than those of the well known alloy containing 8 per cent copper, with the

use of only relatively small amounts of copper or zinc or both. The possibility of limiting these heavy metals to amounts of say 5 per cent or less in the case of copper, and 10 per cent or less in the case of zinc, is very advantageous both as respects the strength of the resulting alloy and as respects its specific gravity. The silicon, by virtue of its lightness, offsets, in a measure, the effect of the heavy metals, copper and zinc, as well as permitting the use of the heavier metals in smaller quantities. We have discovered that these silicon alloys can be materially improved by an appropriate heat treatment, which may affect both the silicon and the heavy-metal constituents.

The tensile strength of commercially pure cast aluminum is about 12,000 pounds per square inch and its elongation about 25 per cent. By adding varying proportions of hardening metals, particularly copper and zinc, it is possible to increase the tensile strength so that the sand cast alloy will have an ultimate strength of nearly 30,000 pounds per square inch, but the elongation is thereby reduced to less than 5 per cent. By adding a very large amount of zinc the tensile strength may be raised to approximately 40,000 pounds per square inch, but the elongation is reduced to almost nothing, and the alloy is very brittle. By casting any of these alloys in a chill mold the tensile strength may be increased in general by approximately 5,000 pounds per square inch and the elongation may also be increased. But it has heretofore been impossible to simultaneously produce tensile strengths of over 30,000 pounds per square inch and an elongation of 8 per cent or over.

By our method, however, we have been able to extend very greatly the range of the tensile strength and elongation, and of the combination of the two, so that we have obtained castings having very much higher tensile strengths than those hitherto known in the art, and yet elongations better than those at present obtained with casting alloys having only moderate tensile strengths.

In general, elongation decreases as tensile strength increases, but our new method enables us to produce very much better simultaneous results in both of these respects than have hitherto been possible.

It is also to be noted that the high tensile

strength alloys previously known have required the presence of substantial amounts of zinc, even in many cases up to 33 per cent, and have therefore been considerably heavier than pure aluminum, while we obtain our results with an addition, in general, of not more than 5 to 10 per cent of total heavier alloying metal or metals and yet produce a casting which is not only stronger and more ductile but likewise lighter than would otherwise be obtained.

Various prior investigators have proposed to obtain castings possessing the desirable combination of high tensile strength and ductility by heat treatment of a properly made casting, but their contributions to the art have so far not led to commercially useful results. For example, the best results published prior to our work are those of Wilm, who reports having obtained castings with a tensile strength of about 32,000 pounds per square inch and an elongation of 5 to 7 per cent. More recently Merica and Karr have by heat treatment of an alloy containing copper and a large amount of zinc, obtained a tensile strength of 41,200 pounds per square inch but with an elongation of only 4 per cent. This alloy contained about 19 per cent of heavy alloying metals and hence had a specific gravity greater than 3. With lighter alloys, for example one containing small amounts of copper, magnesium and manganese, they obtained a tensile strength of 35,500 pounds per square inch and an elongation of 2.3 per cent. In none of the three cases mentioned above were the properties enough better than those possessed by untreated castings to justify the cost of the treatment.

Our invention involves the discovery of important reasons for previous lack of practical success along this line, and embraces a combination of old and new steps so that we are now able by means of our improved method to produce articles, cast in either sand or chill molds, having physical properties far superior to those of any such castings hitherto produced. By means of our novel method we have produced sand castings of an aluminum alloy containing 4 per cent copper and 0.2 per cent magnesium, having a tensile strength of about 50,000 pounds per square inch and an elongation of 8.5 per cent, with relatively high elastic limit; also chilled castings having a tensile strength of 54,000 pounds per square inch and an elongation of 18 per cent, with relatively high elastic limit.

This combination of high tensile strength and elongation enables these castings to be used for purposes for which aluminum castings have not hitherto been suitable and for which it has been necessary to use the much heavier ferrous materials such as steel or malleable iron.

One example of our process comprises as its first step the preparation of an aluminum alloy containing about 3 to 5.5 per cent copper, preferably 4 per cent, with no magnesium or with magnesium up to about 0.3 per cent, the iron content in particular being as low as possible, preferably not to exceed 0.25 per cent. Iron and silicon are always present as impurities in aluminum as now obtainable, and a part of our invention consists in so choosing the raw materials as to limit the iron content of the finished alloy to an amount as low as possible, preferably not over 0.25 per cent. The use of silicon in substantial amounts will be considered here-  
75  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955<br

ture, the time for maximum solution is less,— for example, 7 hours has been found to be sufficient in some cases.

If the copper content exceeds the amount which is soluble in the solid state just below the freezing point of the eutectic, some of the  $\text{CuAl}_2$  will remain in the network after heat treatment, and the physical properties of the casting will not be as good as can be obtained with a lower copper content. In most if not all cases the best combination of physical properties results only when substantially all of the  $\text{CuAl}_2$  in the network has been dissolved in the aluminum-rich constituent.

A temperature of heat-treatment high enough to fuse the eutectic is in most cases unfavorable to the best ultimate results, and it has been found that in some instances 20  $540^\circ \text{C}$ . is too high unless the rate of heating up to that point is very slow or the time of heating below that point is comparatively long.

A further result of heating the castings 25 at the temperature mentioned is to re-dissolve any  $\text{CuAl}_2$ , which may have precipitated in small particles within the aluminum-rich constituent rather than in the network during the previous cooling of the castings.

After the heating period the castings are preferably cooled rapidly, as by quenching in water. By the above described procedure, sand castings of an alloy containing 4 35 per cent copper, 0.2 per cent magnesium and less than .25 per cent iron have been produced with a tensile strength, after aging, of about 50,000 pounds per square inch and an elongation of 8.5 per cent. Chill castings 40 have been made by the same process, of the same alloy, having a tensile strength of 54,000 pounds per square inch after aging and an elongation of 18 per cent.

As stated above, quenching is preferable to 45 slow cooling, but good results can in some cases be obtained by cooling in a current of air. A marked difference has been observed between the results obtained by cooling in a current of air and those obtained by cooling 50 in still air. Even slow cooling, however, produces improvement as compared to the cast condition, not only in the physical properties but also in resistance to corrosion.

The physical properties of castings subjected to the treatments above referred to 55 can be further changed by heating, immediately after cooling, to a temperature of  $100^\circ$  to  $150^\circ \text{C}$ . for a time, one hour being in many cases sufficient. As a result of this 60 heating the tensile strength is increased and the elongation decreased, and the elastic limit is increased very markedly.

The method of casting is an important 65 factor. Thus a method producing fine grain and improved physical properties,

yields castings which are generally more amenable to the heat-treatment than does a casting method which produces coarse grain. For example a bar having a cylindrical test section two inches long and a 70 half-inch in diameter, composed of alloy containing about 4 per cent copper and cast in a sand mold, has a tensile strength of about 18,000 pounds per square inch and an elongation of about 4 per cent. If the 75 bar is heat-treated by our method, say at a temperature around  $520^\circ \text{C}$ . for 24 hours, the tensile strength may be more than doubled (increasing to about 37,000 pounds per square inch) and the elongation is increased 80 to about 12 per cent, or three times its original value. On the other hand, if the bar is cast in such a manner as to cause rapid solidification, say by chill casting in an iron mold, it will have, after heat-treatment 85 by our method, a tensile strength of about 40,000 pounds per square inch, and an elongation of about 20 per cent.

In sand castings of alloys containing substantial amounts of silicon a considerable 90 portion of the latter appears in the form of relatively large plates or needles, and in chill castings the silicon is found generally in smaller particles, some of which at least are more or less rounded. The heat-treatment changes the shape and sometimes the size of the silicon particles, tending toward a more rounded form, and the improvement in physical properties produced by the heat-treatment of such alloys is due in part to 95 this change.

The addition, to the aluminum-copper alloys, of a small amount of magnesium, say 0.2 or 0.3 per cent, increases the tensile 100 strength and elastic limit, but is less favorable to ductility or elongation. Magnesium may also be added to the aluminum-silicon alloys, the effect, generally, being to increase the tensile strength and diminish the elongation.

For the best results, our experience indicates that the iron content of the aluminum copper alloy should be low, but if care is taken to make the castings by the chill 115 method, a higher percentage of iron can be used, good results being obtained with chill castings containing even more than 0.4 per cent of iron. On the other hand, in the case of heat-treated sand castings, more than 120 that amount of iron gives less advantageous physical properties. The presence of the iron is evidenced by crystalline needles, probably of the composition  $\text{FeAl}_3$ , which usually form in the network containing  $\text{CuAl}_2$ . These needles are not soluble to 125 any considerable extent in the solid aluminum alloy, and remain intact and in place while the  $\text{CuAl}_2$  is absorbed into the body of the solid-solution crystals of aluminum during heat-treatment. The iron needles tend 130

to have a beneficial effect on the physical properties of the alloy as cast, that is before heat-treatment, but after the  $\text{CuAl}_2$  in the network has been dissolved into the 5 aluminum-rich constituent by heat-treating, the iron needles are a source of weakness, diminishing both tensile strength and elongation.

The complete elimination of the iron needles is therefore highly desirable, but the complete avoidance of iron or even its reduction below about 0.25 per cent is not always practicable commercially. However, when silicon is present in excess of the 15 iron, the quantity of  $\text{FeAl}_3$  formed is lessened, and some of the iron combines with the silicon to form what appears to be an iron silicide. We have discovered that the latter compound freezes in a form less 20 harmful than the needles of  $\text{FeAl}_3$ . In the case of chill castings, it is found that the  $\text{FeAl}_3$  needles are much smaller than in the sand castings, and hence they are not so objectionable in the heat-treated casting. 25 Since there is considerable difficulty in commercially producing aluminum free from or containing less than 0.25 per cent of iron, the desired silicon-iron relationship is most advantageously obtained by adding silicon 30 when necessary. For example, if the iron content of the aluminum ingot is 0.35 per cent and the silicon 0.3 per cent, we find it advantageous to add about 0.35 per cent silicon. We have also found that the addition 35 of a small quantity of zinc, say 0.25 per cent, improves both the tensile strength and elongation of the heat-treated castings.

Chromium up to 0.5 per cent or a little 40 more increases the tensile strength in the heat-treated casting, but reduces the elongation.

With regard to the limits of copper content, we have observed that up to about 2 per cent copper, nearly all the  $\text{CuAl}_2$  45 remains in solution upon solidification, and that beyond 5.5 per cent copper some of the  $\text{CuAl}_2$  usually remains out of solution even after heat-treatment. In some cases the metal can be heated above the melting point 50 of the eutectic of  $\text{CuAl}_2$  and aluminum without impairing its physical properties provided the metal is cooled to a temperature slightly below that of complete solidification and held there for some time before 55 quenching. When substantial percentages of iron, silicon, magnesium and zinc are present, or any of them, the higher permissible temperature is lowered.

A very important class of alloys embraced 60 by our invention includes the use of silicon in substantial amount, say from 3 to 15 per cent. With the silicon class of alloys the best results are usually obtained when the castings are made in a chill mold. For ex-

ample, a chill cast test bar of an alloy containing about 10 per cent silicon and no copper showed a tensile strength around 30,000 pounds per square inch and an elongation of about 7.5 per cent in two inches. After heating at 560° C. for 40 hours, followed by quenching, the tensile strength was about 27,500 pounds per square inch, but the elongation was found to have been increased to 21 per cent. We are therefore able to produce by our method a casting of aluminum-silicon alloy having great ductility and at the same time a tensile strength twice or more than twice that of aluminum, with the further advantage of good casting qualities as mentioned above. The addition of 75 copper to this aluminum-silicon alloy increases the tensile strength enormously but decreases the elongation. Chill cast bars of an alloy containing 6 per cent silicon and 4 per cent copper, heated 45 hours at 500 to 80 515° C. followed by quenching, showed a tensile strength as high as 42,000 pounds per square inch and an elongation of 8 per cent. In the high silicon alloys the most advantageous copper content is from 2 to 5 per cent. It should be noted that the eutectic of the aluminum-silicon system melts at 570 to 580° C., which is higher than the melting point of the aluminum-copper eutectic 85 which is at 540° C. and therefore it is not only permissible but advantageous to heat-treat the former alloys at higher temperatures,—say 530 to 570° C. When copper is added to the aluminum-silicon alloys a ternary eutectic may form with a melting point of about 520° C. and consequently the heat-treatment temperature should be lowered accordingly. Zinc and magnesium also 90 lower the maximum heat-treating temperature of the aluminum-silicon alloys. 100

Zinc can also be added to the aluminum alloys containing substantial amounts of silicon and copper or either of them. For example an alloy containing 8 per cent silicon, 10 per cent zinc and 2.5 per cent copper, gave a tensile strength of 32,300 pounds per square inch, and an elongation of 2.5 per cent in 2 inches in a chill cast test bar, and after heat-treatment similar to that mentioned above the tensile strength was increased to over 44,000 pounds per square inch and the elongation to 7 per cent. In case only silicon and zinc are present, it is found that the heat treatment has a less beneficial effect on the tensile strength, but the elongation is very favorably affected. For example, in an alloy containing 8 per cent silicon and 10 per cent zinc, a chill cast test bar gave a tensile strength of 29,250 pounds per square inch and an elongation of 4 per cent, whereas after heat treatment the tensile strength was 30,500 pounds per square inch and the elongation had increased to 1125 115 120 125

per cent. It is also found that the heat-treatment can be used in conjunction with the process for improving the physical properties of these alloys by the addition of alkali metals to the molten alloy, as described in the patent of Junius D. Edwards, Francis C. Frary and Harry V. Churchill, No. 1,410,461, issued March 21, 1922, on their application Serial No. 426,796, copending herewith. For example, chill cast test bars of an alloy containing 8 per cent silicon and 10 per cent zinc, to which alkali metals were added before pouring, gave an average tensile strength of over 41,000 pounds per square inch and an elongation of 6.2 per cent in 2 inches. Heat-treatment reduced the tensile strength to 34,000 pounds per square inch, but increased the elongation to 14 per cent.

20 To obtain the best results it is desirable, in all the above mentioned aluminum-silicon alloys, to keep the iron content low, preferably below 0.6 per cent.

It is found that the coarser the grain produced in casting, the longer must the heat-treatment be continued to produce the most beneficial results. Accordingly sand castings with large cross-sectional areas require longer heating than chill castings. Usually 30 holding at temperature for about 7 hours is sufficient for chill castings, whereas 24 hours may be necessary with sand castings.

In addition to the production of a superior grade of sand castings, permanent mold or chill castings (including die castings), the application of our invention is also most important in connection with the forging and pressing of aluminum alloys. If it is desired to produce a forging of a given 40 shape, a casting of suitable composition, say 4 per cent copper and 0.2 per cent magnesium, is made, preferably in a chill mold, and is subjected to heat-treatment by our method to produce a starting material for 45 forging.

In this case, instead of quenching from the heat-treatment temperature and then reheating the article to forging temperature, we find it preferable to simply cool slowly 50 from the heat-treatment temperature to the forging temperature. The piece is then finished to size under the press or hammer, after which it is given a short heating, say at 520° C., followed by quenching.

55 The duration of the heat-treatment step of our method depends, in large measure, other conditions being the same, upon the degree of improvement desired in the physical properties of the casting.

60 The essential thing to be kept in mind is the relatively long time required for cast alloys in general, as compared to those rolled aluminum-copper alloys known to the prior heat-treating art. This is caused, in the

case of the cast copper alloys, by the greater 65 difficulty in getting the unbroken CuAl<sub>2</sub> network into solution in the aluminum, and in the case of the silicon alloys by the slowness of change of form of the silicon. In case both copper and silicon are present in 70 substantial quantities, time must be allowed for both of these changes to take place to the extent necessary for the desired improvement.

In the copper alloys containing about 4 75 per cent copper, for example, it is found that heating for very long periods, say 48 hours or more, at temperatures only slightly below 500° C. will not, in general, produce as good results as a five hour treatment at 80 520° C. In chill castings of the copper alloys it has been found that even two hours heating at 520° C. produced substantially as good results as about 22 hours at 500° C. In order to reduce the time to a minimum, we 85 prefer, if suitable temperature control is available, to use as high a temperature as can be safely employed without spoiling the castings by overheating.

We have also found that in the case of 90 alloy containing substantial amounts of silicon, the change in shape of the silicon particles is effected more quickly and more completely at relatively high temperatures. In these alloys, heating for about 12 hours 95 at 520° C. produces very substantial improvement, but the time may be extended, with slight additional improvement, if desired. At a temperature of 550 to 570° C. the aluminum-silicon alloys may be heat-treated with more beneficial results than can be produced at 500° C. or thereabouts. 100

It is to be understood that the invention is not limited to the specific details herein described but can be practised in other ways 105 without departure from its spirit.

We claim:

1. In the art of making aluminum alloy castings, the method comprising heating an alloy casting containing a substantial amount of silicon, to a temperature slightly below the melting point of the eutectic, and maintaining such temperature until the silicon particles have been sufficiently altered 110 in shape to materially improve the physical properties of the cast alloy. 115

2. In the art of making aluminum alloy castings, the method comprising preparing an alloy containing a substantial amount of silicon, casting the alloy and causing the silicon therein to take the form of relatively small particles in the solidified alloy, heating the casting to a temperature slightly below the melting point of the eutectic, and maintaining such temperature until the silicon particles have been sufficiently altered 120 to materially improve the physical properties of the cast alloy. 125

3. In the art of making aluminum alloy castings, the method comprising preparing an alloy containing a substantial amount of silicon, chill casting the alloy whereby the silicon is caused to take the form of relatively small particles in the solidified alloy, heating the casting to a temperature slightly below the melting point of the eutectic, and maintaining such temperature until the silicon particles have been sufficiently altered in shape to materially improve the physical properties of the alloy.

4. In the art of making aluminum alloy castings, the method comprising heating an alloy casting containing from 3 to 15 per cent silicon, to a temperature slightly below the melting point of the eutectic, and maintaining such temperature until the silicon particles have been sufficiently altered in shape to materially improve the physical properties of the cast alloy.

5. In the art of making aluminum alloy castings, the method comprising preparing an alloy containing 3 to 15 per cent silicon, casting the alloy and causing the silicon therein to take the form of relatively small particles, heating the casting to a temperature slightly below the melting point of the eutectic, and maintaining such temperature until the silicon particles have been sufficiently altered to materially improve the physical properties of the cast alloy.

6. In the art of making aluminum alloy castings, the method comprising heating an alloy casting containing from 8 to 10 per cent silicon, to a temperature slightly below the melting point of the eutectic, and maintaining such temperature until the silicon particles have been sufficiently altered in shape to materially improve the physical properties of the cast alloy.

7. In the art of making aluminum alloy castings, the method comprising heating an alloy casting containing a substantial amount of silicon and not more than about 0.6 per cent of iron, to a temperature slightly below the melting point of the eutectic, and maintaining such temperature until the silicon particles have been sufficiently altered in shape to materially improve the physical properties of the cast alloy.

8. In the art of making aluminum alloy castings, the method comprising heating an alloy casting containing a substantial amount of silicon, at a temperature slightly below the melting point of the eutectic until the silicon particles have been sufficiently altered in shape to materially improve the physical properties of the cast alloy, and cooling the casting rapidly.

9. In the art of making aluminum alloy castings, the method comprising preparing an alloy containing a substantial amount of silicon, casting the alloy and causing the silicon therein to take the form of relatively

small particles in the solidified alloy, heating the casting at a temperature slightly below the melting point of the eutectic until the silicon particles have been sufficiently altered to materially improve the physical properties of the cast alloy, and cooling the casting rapidly.

10. In the art of making aluminum alloy castings, the method comprising preparing an alloy containing a substantial amount of silicon, chill casting the alloy whereby the silicon is caused to take the form of relatively small particles in the solidified alloy, heating the casting at a temperature slightly below the melting point of the eutectic until the silicon particles have been sufficiently altered in shape to materially improve the physical properties of the alloy, and cooling the casting rapidly.

11. In the art of making aluminum alloy castings, the method comprising heating an alloy casting containing from 3 to 15 per cent silicon, at a temperature slightly below the melting point of the eutectic until the silicon particles have been sufficiently altered in shape to materially improve the physical properties of the cast alloy, and cooling the casting rapidly.

12. In the art of making aluminum alloy castings, the method comprising preparing an alloy containing 3 to 15 per cent silicon, casting the alloy and causing the silicon therein to take the form of relatively small particles, heating the casting at a temperature slightly below the melting point of the eutectic until the silicon particles have been sufficiently altered to materially improve the physical properties of the cast alloy, and cooling the casting rapidly.

13. In the art of making aluminum alloy castings, the method comprising heating an alloy casting containing from 8 to 10 per cent silicon, at a temperature slightly below the melting point of the eutectic until the silicon particles have been sufficiently altered in shape to materially improve the physical properties of the cast alloy, and cooling the casting rapidly.

14. In the art of making aluminum alloy castings, the method comprising heating an alloy casting containing a substantial amount of silicon and not more than about 0.6 per cent of iron, at a temperature slightly below the melting point of the eutectic until the silicon particles have been sufficiently altered in shape to materially improve the physical properties of the cast alloy, and cooling the casting rapidly.

15. In the art of making aluminum alloy castings, the method comprising heating an alloy casting containing substantial amounts of silicon and copper, casting the alloy, heating the casting to a temperature slightly below the melting point of the eutectic, and maintaining such temperature until the sil-

icon particles have been sufficiently altered in shape and a sufficient amount of the inter-granular copper-rich constituent has been dissolved to materially improve the physical properties of the cast alloy.

16. In the art of making aluminum alloy castings, the method comprising preparing an alloy containing substantial amounts of silicon and copper, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

17. In the art of making aluminum alloy castings, the method comprising heating an alloy casting containing substantial amounts of silicon and copper, at a temperature slightly below the melting point of the eutectic until the silicon particles have been sufficiently altered and a sufficient amount of the intergranular copper-rich constituent has been dissolved to materially improve the physical properties of the cast alloy, and cooling the casting rapidly.

18. In the art of making aluminum alloy castings, the method comprising preparing an alloy containing substantial amounts of silicon and copper, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

19. In the art of making aluminum alloy castings, the method comprising heating an alloy casting containing a substantial amount of copper and 3 to 15 per cent silicon, at a temperature slightly below the melting point of the eutectic until the silicon particles have been sufficiently altered in shape and a sufficient amount of the inter-granular copper-rich constituent has been dissolved to materially improve the physical properties of the cast alloy.

20. In the art of making aluminum alloy castings, the method comprising heating an alloy casting containing a substantial amount of copper and 3 to 15 per cent silicon, at a temperature slightly below the melting point of the eutectic until the silicon particles have been sufficiently altered in shape and a sufficient amount of the inter-granular copper-rich constituent has been dissolved to materially improve the physical properties

of the cast alloy, and cooling the casting rapidly.

21. In the art of making aluminum alloy castings, the method comprising preparing an alloy containing a substantial amount of copper and 3 to 15 per cent silicon, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

22. In the art of making aluminum alloy castings, the method comprising preparing an alloy containing a substantial amount of copper and 3 to 15 per cent silicon, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

23. In the art of making aluminum alloy castings, the method comprising heating an alloy casting containing substantial amounts of silicon and copper and having a low iron content, to a temperature slightly below the melting point of the eutectic, and maintaining such temperature until the silicon particles have been sufficiently altered in shape and a sufficient amount of the inter-granular copper-rich constituent has been dissolved to materially improve the physical properties of the cast alloy.

24. In the art of making aluminum alloy castings, the method comprising preparing an alloy containing substantial amounts of silicon and copper and having a low iron content, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

25. In the art of making aluminum alloy castings, the method comprising heating an alloy casting containing substantial amounts of silicon and copper and having a low iron content, at a temperature slightly below the melting point of the eutectic until the sili-

con particles have been sufficiently altered and a sufficient amount of the inter-granular copper-rich constituent has been dissolved to materially improve the physical properties of the cast alloy, and cooling the casting rapidly.

26. In the art of making aluminum alloy castings, the method comprising preparing an alloy containing substantial amounts 10 of silicon and copper and having a low iron content, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical 15 properties of the cast alloy, and cooling the casting rapidly.

27. In the art of making aluminum alloy castings, the method comprising heating an alloy casting containing a substantial 25 amount of copper and 3 to 15 per cent silicon, and having a low iron content, casting the alloy, heating the casting at a temperature slightly below the melting point of the eutectic until the silicon particles have 30 been sufficiently altered and a sufficient amount of the inter-granular copper-rich constituent has been dissolved to materially improve the physical properties of the cast alloy, and cooling the casting rapidly.

28. In the art of making aluminum alloy castings, the method comprising preparing an alloy containing a substantial amount of copper and 3 to 15 per cent silicon, and having a low iron content; casting the alloy 35 and causing the silicon therein to take the form of relatively small particles in the solidified alloy, heating the casting to a temperature slightly below the melting point of the eutectic, and maintaining such 40 temperature until the silicon particles have been sufficiently altered and a sufficient amount of the inter-granular copper-rich constituent has been dissolved to materially improve the physical properties of the cast alloy, and cooling the casting rapidly.

29. In the art of making aluminum alloy castings, the method comprising preparing an alloy containing a substantial amount of copper and 3 to 15 per cent silicon, and 45 having a low iron content; casting the alloy and causing the silicon therein to take the form of relatively small particles in the solidified alloy, heating the casting at a temperature slightly below the melting point 50 of the eutectic until the silicon particles have been sufficiently altered and a sufficient amount of the inter-granular copper-rich constituent has been dissolved to materially improve the physical properties of the cast alloy, and cooling the casting rapidly.

30. In the art of making aluminum alloy castings, the method comprising heating an alloy casting containing 2 to 5.5 per cent copper and a substantial amount of silicon, to a temperature slightly below the melting point of the eutectic, and maintaining such temperature until the silicon particles have been sufficiently altered in shape and a sufficient amount of the inter-granular copper-rich constituent has been dissolved to materially improve the physical properties of the cast alloy. 70

31. In the art of making aluminum alloy castings, the method comprising preparing an alloy containing 2 to 5.5 per cent copper and a substantial amount of silicon, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy. 80

32. In the art of making aluminum alloy castings, the method comprising heating an alloy casting containing 2 to 5.5 per cent copper and a substantial amount of silicon, at a temperature slightly below the melting point of the eutectic until the silicon particles have been sufficiently altered and a sufficient amount of the inter-granular copper-rich constituent has been dissolved to materially improve the physical properties of the cast alloy. 90

33. In the art of making aluminum alloy castings, the method comprising preparing an alloy containing 2 to 5.5 per cent copper and a substantial amount of silicon, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly. 100

34. In the art of making aluminum alloy castings, the method comprising heating an alloy casting containing 2 to 5.5 per cent copper and 3 to 15 per cent silicon, at a temperature slightly below the melting point of the eutectic until the silicon particles have been sufficiently altered in shape and a sufficient amount of the inter-granular copper-rich constituent has been dissolved to materially improve the physical properties of the cast alloy. 110

120

125

130

35. In the art of making aluminum alloy castings, the method comprising heating an alloy casting containing 2 to 5.5 per cent copper and 3 to 15 per cent silicon, at a temperature slightly below the melting point of the eutectic until the silicon particles have been sufficiently altered in shape and a sufficient amount of the inter-granular copper-rich constituent has been dissolved to materially improve the physical properties of the cast alloy, and cooling the casting rapidly.

36. In the art of making aluminum alloy castings, the method comprising preparing an alloy containing 2 to 5.5 per cent copper and 3 to 15 per cent silicon, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

37. In the art of making aluminum alloy castings, the method comprising preparing an alloy containing 2 to 5.5 per cent copper and 3 to 15 per cent silicon, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy.

38. In the art of making aluminum alloy castings, the method comprising heating an alloy casting containing 2 to 5.5 per cent copper and a substantial amount of silicon, and having a low iron content, to a temperature slightly below the melting point of the eutectic, and maintaining such temperature until the silicon particles have been sufficiently altered in shape and a sufficient amount of the inter-granular copper-rich constituent has been dissolved to materially improve the physical properties of the cast alloy.

39. In the art of making aluminum alloy castings, the method comprising preparing an alloy containing 2 to 5.5 per cent copper and a substantial amount of silicon, and having a low iron content, casting the alloy, and causing the silicon therein to take the form of relatively small particles in the solidified alloy, heating the casting to a temperature slightly below the melting point of the eutectic, and maintaining such temperature until the silicon particles have been

sufficiently altered and a sufficient amount of the inter-granular copper-rich constituent has been dissolved to materially improve the physical properties of the cast alloy.

40. In the art of making aluminum alloy castings, the method comprising heating an alloy casting containing 2 to 5.5 per cent copper and a substantial amount of silicon, and having a low iron content, casting the alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

41. In the art of making aluminum alloy castings, the method comprising preparing an alloy containing 2 to 5.5 per cent copper and a substantial amount of silicon, and having a low iron content, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

42. In the art of making aluminum alloy castings, the method comprising heating an alloy casting containing 2 to 5.5 per cent copper and 3 to 15 per cent silicon, and having a low iron content, at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

43. In the art of making aluminum alloy castings, the method comprising preparing an alloy containing 2 to 5.5 per cent copper and 3 to 15 per cent silicon, and having a low iron content; casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

44. In the art of making aluminum alloy castings, the method comprising preparing an alloy containing 2 to 5.5 per cent copper and 3 to 15 per cent silicon, and having a low iron content; casting the alloy

- and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.
45. In the art of making aluminum alloy castings, the method comprising heating an alloy casting containing 3 to 10 per cent silicon and a substantial amount of copper, at a temperature slightly below the melting point of the eutectic until the silicon particles have been sufficiently altered in shape and a sufficient amount of the inter-granular copper-rich constituents has been dissolved to materially improve the physical properties of the cast alloy.
46. In the art of making aluminum alloy castings, the method comprising heating an alloy casting containing 3 to 10 per cent silicon and a substantial amount of copper, at a temperature slightly below the melting point of the eutectic until the silicon particles have been sufficiently altered in shape and a sufficient amount of the inter-granular copper-rich constituent has been dissolved to materially improve the physical properties of the cast alloy, and cooling the casting rapidly.
47. In the art of making aluminum alloy castings, the method comprising preparing an alloy containing 3 to 10 per cent silicon and a substantial amount of copper, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.
50. 48. In the art of making aluminum alloy castings, the method comprising preparing an alloy containing 3 to 10 per cent silicon and a substantial amount of copper, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.
49. In the art of making aluminum alloy castings, the method comprising heating an alloy casting containing 3 to 10 per cent silicon and a substantial amount of copper, and having an iron content not exceeding about 0.6 per cent, at a temperature slightly below the melting point of the eutectic until the silicon particles have been sufficiently altered in shape and a sufficient amount of the inter-granular copper-rich constituent has been dissolved to materially improve the physical properties of the cast alloy.
50. In the art of making aluminum alloy castings, the method comprising heating an alloy casting containing 3 to 10 per cent silicon and a substantial amount of copper, and having an iron content not exceeding about 0.6 per cent, at a temperature slightly below the melting point of the eutectic until the silicon particles have been sufficiently altered in shape and a sufficient amount of the inter-granular copper-rich constituent has been dissolved to materially improve the physical properties of the cast alloy, and cooling the casting rapidly.
51. In the art of making aluminum alloy castings, the method comprising preparing an alloy containing 3 to 10 per cent silicon and a substantial amount of copper, and having an iron content not exceeding about 0.6 per cent; casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.
52. In the art of making aluminum alloy castings, the method comprising preparing an alloy containing 3 to 10 per cent silicon and a substantial amount of copper, and having an iron content not exceeding about 0.6 per cent; casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.
53. In the art of making aluminum alloy castings, the method comprising heating an alloy casting containing copper 4 per cent and silicon 6 per cent, approximately, at a temperature slightly below the melting point of the eutectic until the silicon particles have been sufficiently altered in shape and a sufficient amount of the inter-granular copper-rich constituent has been dis-

solved to materially improve the physical properties of the cast alloy.

54. In the art of making aluminum alloy castings, the method comprising heating an alloy casting containing 4 per cent copper and 6 per cent silicon, approximately, at a temperature slightly below the melting point of the eutectic until the silicon particles have been sufficiently altered in shape and a sufficient amount of the inter-granular copper-rich constituent has been dissolved to materially improve the physical properties of the cast alloy, and cooling the casting rapidly.
- 10 55. In the art of making aluminum alloy castings, the method comprising preparing an alloy containing 4 per cent copper and 6 per cent silicon, approximately, casting the alloy and causing the silicon therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.

56. In the art of making aluminum alloy castings, the method comprising preparing an alloy containing 4 per cent copper and 6 per cent silicon, approximately, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy and cooling the casting rapidly.

57. In the art of making aluminum alloy castings, the method comprising heating an alloy casting containing substantial amounts of silicon and copper and a relatively small amount of magnesium, to a temperature slightly below the melting point of the eutectic, and maintaining such temperature until the silicon particles have been sufficiently altered in shape and a sufficient amount of the inter-granular copper-rich constituent has been dissolved to materially improve the physical properties of the cast alloy.

58. In the art of making aluminum alloy castings, the method comprising preparing an alloy containing substantial amounts of silicon and copper and a relatively small amount of magnesium, casting the alloy and causing the silicon therein to take the form of relatively small particles in the solidified alloy, heating the casting to a temperature slightly below the melting point of the eutectic, and maintaining such temperature

until the silicon particles have been sufficiently altered and a sufficient amount of the inter-granular copper-rich constituent has been dissolved to materially improve the physical properties of the cast alloy.

59. In the art of making aluminum alloy castings, the method comprising heating an alloy casting containing substantial amounts of silicon and copper and a relatively small amount of magnesium, at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

60. In the art of making aluminum alloy castings, the method comprising preparing an alloy containing substantial amounts of silicon and copper and a relatively small amount of magnesium, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.

61. In the art of making aluminum alloy castings, the method comprising heating an alloy casting containing a substantial amount of copper and 3 to 15 per cent silicon, and a relatively small amount of magnesium, casting the alloy, and heating the casting at a temperature slightly below the melting point of the eutectic until the silicon particles have been sufficiently altered in shape and a sufficient amount of the inter-granular copper-rich constituent has been dissolved to materially improve the physical properties of the cast alloy.

62. In the art of making aluminum alloy castings, the method comprising heating an alloy casting containing a substantial amount of copper and 3 to 15 per cent silicon, and a relatively small amount of magnesium, casting the alloy, heating the casting at a temperature slightly below the melting point of the eutectic until the silicon particles have been sufficiently altered in shape and a sufficient amount of the inter-granular copper-rich constituent has been dissolved to materially improve the physical properties of the cast alloy, and cooling the casting rapidly.

63. In the art of making aluminum alloy castings, the method comprising preparing an alloy containing a substantial amount of copper and 3 to 15 per cent silicon, and a relatively small amount of magnesium, casting the alloy and causing the silicon

- therein to take the form of relatively small particles in the solidified alloy, heating the casting to a temperature slightly below the melting point of the eutectic, and maintaining such temperature until the silicon particles have been sufficiently altered and a sufficient amount of the inter-granular copper-rich constituent has been dissolved to materially improve the physical properties of the cast alloy.
64. In the art of making aluminum alloy castings, the method comprising preparing an alloy containing a substantial amount of copper and 3 to 15 per cent silicon, and a relatively small amount of magnesium, casting the alloy and causing the silicon therein to take the form of relatively small particles in the solidified alloy, heating the casting at a temperature slightly below the melting point of the eutectic until the silicon particles have been sufficiently altered and a sufficient amount of the inter-granular copper-rich constituent has been dissolved to materially improve the physical properties of the cast alloy, and cooling the casting rapidly.
65. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy; heating the casting at a temperature between about 500° C. and about 540° C., for a relatively long period of time, until a sufficient amount of the inter-granular copper-rich constituent has been dissolved to materially improve the physical properties of the cast alloy.
66. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy; and heating the casting at a temperature between about 500° C. and about 540° C. for not less than about two hours, until a sufficient amount of the inter-granular copper-rich constituent has been dissolved to materially improve the physical properties of the cast alloy.
67. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy and causing rapid solidification there-
- of in the mold; and heating the casting at a temperature between about 500° C. and about 540° C. for a relatively long period of time, until a sufficient amount of the inter-granular copper-rich constituent has been dissolved to materially improve the physical properties of the cast alloy.
68. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy and causing rapid solidification thereof in the mold; and heating the casting at a temperature between about 500° C. and about 540° C. for not less than about 2 hours, until a sufficient amount of the inter-granular copper-rich constituent has been dissolved to materially improve the physical properties of the cast alloy.
69. In the art of making aluminum alloy castings, the method comprising preparing an alloy containing 0.25 per cent zinc and 4 per cent copper, approximately, magnesium not exceeding about 0.3 per cent, iron not exceeding about 0.4 per cent, and silicon in excess of the iron, and in preparing the alloy keeping the temperature not greatly in excess of 750° C.; casting the alloy; heating the casting at a temperature between about 500° C. and about 540° C., for a relatively long period of time, until a sufficient amount of the inter-granular copper-rich constituent has been dissolved to materially improve the physical properties of the cast alloy.
70. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy, heating the casting at a temperature between about 500° C. and 540° C., for a relatively long period of time, until a sufficient amount of the inter-granular copper-rich constituent has been dissolved to materially improve the physical properties of the cast alloy, and cooling the casting rapidly.
71. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy, heating the casting at a temperature between about 500° C. and about 540° C. for not less than about 2 hours, until a sufficient

amount of the inter-granular copper-rich constituent has been dissolved to materially improve the physical properties of the cast alloy, and cooling the casting rapidly.

5 72. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy and causing rapid solidification thereof in the mold; heating the casting at a temperature between about 500° C. and about 540° C., for a relatively long period of time, until a sufficient amount of the inter-granular copper-rich constituent has been dissolved to materially improve the physical properties of the cast alloy, and cooling the casting rapidly.

25 73. In the art of making aluminum alloy castings, the method comprising preparing an alloy containing about 4 per cent copper, magnesium not exceeding about 0.3 per cent, iron not exceeding about 0.4 per cent, and silicon in excess of the iron, and in preparing the alloy keeping the temperature not greatly in excess of 750° C.; casting the alloy and causing rapid solidification thereof in the mold; heating the casting at a temperature between about 500° C. and about 540° C. for not less than about 2 hours, until a sufficient amount of the inter-granular copper-rich constituent has been dissolved to materially improve the physical properties of the cast alloy, and cooling the casting rapidly.

30 74. As a new article of manufacture, a heat-treated casting of an aluminum alloy containing a substantial amount of silicon, characterized by the silicon being in the form of small finely dispersed more or less rounded particles and substantially devoid of large plates and needles of silicon, with consequent high tensile strength and elongation.

35 75. As a new article of manufacture, a heat-treated casting of an aluminum alloy containing silicon in amount between 3 and 15 per cent, characterized by the silicon being in the form of small finely dispersed more or less rounded particles and substantially devoid of large plates and needles of silicon, with consequent high tensile strength and elongation.

76. As a new article of manufacture, a heat-treated casting of an aluminum alloy containing substantial amounts of silicon and copper, characterized by the silicon being in the form of small finely dispersed more or less rounded particles and substantially devoid of large silicon plates or needles and of undissolved inter-granular copper-rich constituent, with consequent high tensile strength and elongation.

77. As a new article of manufacture, a heat-treated casting of an aluminum alloy containing a substantial amount of silicon and having a low iron content, characterized by the silicon being in the form of small finely dispersed more or less rounded particles and substantially devoid of large plates and needles of silicon, with consequent high tensile strength and elongation.

78. As a new article of manufacture, a heat-treated casting of an aluminum alloy containing silicon in amount between 3 and 15 per cent and having a low iron content, characterized by the silicon being in the form of small finely dispersed more or less rounded particles and substantially devoid of large silicon plates or needles of silicon, with consequent high tensile strength and elongation.

79. As a new article of manufacture, a heat-treated casting of an aluminum alloy containing substantial amounts of silicon and copper and a relatively small amount of magnesium, and having a low iron content, characterized by the silicon being in the form of small finely dispersed more or less rounded particles and substantially devoid of large silicon plates or needles and of undissolved inter-granular copper-rich constituent, with consequent high tensile strength and elongation.

80. As a new article of manufacture, a heat-treated casting of an aluminum alloy containing substantial amounts of silicon and copper and a relatively small amount of magnesium, characterized by the silicon being in the form of small finely dispersed more or less rounded particles and substantially devoid of large silicon plates or needles and of undissolved inter-granular copper-rich constituent, with consequent high tensile strength and elongation.

In testimony whereof we hereto affix our signatures.

ZAY JEFFRIES.  
ROBERT S. ARCHER.

**Certificate of Correction.**

It is hereby certified that in Letters Patent No. 1,508,556, granted September 16, 1924, upon the application of Zay Jefferies, of Cleveland Heights, and Robert S. Archer, of East Cleveland, Ohio, for an improvement in "Making Castings of Aluminum Alloys," errors appear in the printed specification requiring correction as follows: Page 6, lines 127 and 128, claim 15; page 8, lines 26 and 27, claim 27; page 9, lines 74 and 75, claim 40, and page 11, lines 116 and 117, claim 62, strike out the words "casting the alloy, heating the casting"; page 11, lines 103 and 104, claim 61, strike out the words "casting the alloy, and heating the casting"; and that the said Letters Patent should be read with these corrections therein that the same may conform to the record of the case in the Patent Office.

Signed and sealed this 28th day of April, A. D. 1925.

[SEAL.]

**KARL FENNING.**